

## UNITED STATES PATENT OFFICE

2,388,833

## YARN TREATING PROCESS AND RESULTING PRODUCT

Joseph B. Dickey, Rochester, N. Y., and James G. McNally, Knoxville, Tenn., assignors to Eastman Kodak Company, Rochester, N. Y., a corporation of New Jersey

No Drawing. Application January 7, 1944.  
Serial No. 517,430

6 Claims. (Cl. 117—139.5)

This invention relates to the conditioning of textile yarns, and particularly to the conditioning of yarns, threads, filaments and fibers composed of or containing organic derivatives of cellulose such as cellulose acetate, cellulose acetate propionate and cellulose acetate butyrate, to render such materials amenable to various textile operations such as knitting, weaving, carding, spinning, twisting and the like.

As is well known in the textile industry, the manufacture, processing and use of yarns composed of or containing organic derivatives of cellulose and similar synthetic materials give rise to numerous problems generally absent from the handling of natural yarns such as silk, wool, cotton, and the like. One of the chief problems encountered in dealing with these synthetic materials is to so lubricate or soften and, in some instances, to both lubricate and soften, the yarn in question that it will have the correct frictional characteristics, or drag, and the required flexibility for the specific purpose in view. In the handling of continuous filament yarn, for example, it is necessary to condition the material to reduce the tendency toward breakage of individual filaments when the yarn is subjected to mechanical strains such as are involved in passage of the yarn over rolls, guides, and other parts of the yarn-producing mechanism and in twisting, winding, reeling and similar operations. In the case of yarns intended for use on commercial knitting machinery, it is particularly important that the yarn be soft and pliable in order that it may conform to the contour of the needles and give a closely knit fabric free from cuts, pinholes, stitch distortion, laddering, mis-plaits and other common defects.

Another problem of major proportions presented by these synthetic yarns is their extreme tendency to pick up charges of static electricity, especially in such operations as twisting, winding, warping, picking, carding, combing, drafting, spinning, and the like. This tendency is particularly aggravated in the case of cut staple fibers, since in the commercial use of such material it is normally subjected to a number of extremely severe operations such as picking, carding, combing, etc., all of which tend to so charge the individual fibers as to make proper web formation difficult or impossible or to give the ultimate yarn an undesirable unevenness.

In some types of yarn, all three of the above-mentioned problems of lubrication, softening and anti-static treatment are present and in any case the matter of providing a yarn condition-

ing composition, in which the several functions are properly coordinated to accomplish the desired result is often a matter of extreme difficulty. This is due to the fact that in any given yarn conditioning composition, whether primarily designed for use as a warp, filling or knitting lubricant, or as an anti-static, all of the various components and their functions must be delicately balanced one against the other so as to give a practical and commercially satisfactory yarn treatment.

Heretofore, many different conditioning agents such as polyhydric alcohols and similar compounds have been suggested as ingredients of yarn conditioning formulas, generally in conjunction with mineral, vegetable and animal oils. It has been found in practice, however, that most of these agents and the various formulas containing them have certain drawbacks, among which may be mentioned too drastic solvent action on the yarn, insufficient solvent power for or solubility in the lubricants with which they are used and a tendency to form gummy deposits on the yarn after application. Furthermore, many of the known lubricating, softening and anti-static agents are insufficiently soluble in water to permit satisfactory removal from the yarn by aqueous scour baths.

The present invention has as its principal object to provide an improved process for the conditioning of textile yarns, threads, filaments, and fibers, particularly those composed of or containing organic derivatives of cellulose to render such materials amenable to various textile operations and processes, such as knitting, weaving, spinning, and the like. A further object is to provide an improved process for the lubrication, softening and anti-static treatment of such yarn. A still further object is to provide a new class of yarn treating agents and compositions particularly adapted for the conditioning of yarns composed of or containing organic derivatives of cellulose and readily removable therefrom by the usual aqueous scourbaths. A specific object is to provide an improved type of cellulose organic derivative cut staple fiber amenable to carding, drawing, spinning, and other processing steps customarily employed in the manufacture of spun yarn on the woolen, worsted, and cotton systems. Other objects will appear hereinafter.

These objects are accomplished by the following invention which, in its broader aspects, comprises treating yarns, particularly those composed of or containing organic derivatives of cellulose, such as cellulose acetate, cellulose

acetate propionate, cellulose acetate butyrate and similar organic acid esters with a carboxylic amide having the formula



wherein Ac is an acyl group,  $\text{R}_1$  is a member of the group consisting of furfuryl and tetrahydrofurfuryl groups and  $\text{R}_2$  is a member of the group consisting of hydrogen, alkyl, hydroxyalkyl, furfuryl and tetrahydrofurfuryl groups. The acyl group may be derived from any aliphatic or aromatic acid. The alkyl group may be any substituted or unsubstituted alkyl.

The preparation and characteristics of this class of carboxylic amides will be more fully illustrated by the following examples and description in which we have set forth several of the preferred embodiments of our invention which are included merely for purposes of illustration and not as a limitation thereof.

#### PREPARATION OF COMPOUNDS

The compounds covered by the graphic formula given above may be prepared, for example, by reacting an appropriate furfurylamine or tetrahydrofurfurylamine with the appropriate acid or acid chloride. The acids we prefer to employ are those typified by stearic, oleic, ricinoleic, palmitic, lauric, sebacic, myristic, abietic, benzoic, naphthenic and the like. These may, in general, be derived from naturally-occurring oils such as olive, neat's-foot, cotton seed, soya bean, whale, jojoba, egg, menhaden and other oils. For example, I may prepare nitrogen-furfuryl palmityl amide by causing furfurylamine to react with palmitic acid or palmityl chloride. Practically any amide may be similarly prepared by procedures typified by those illustrated in the following examples.

The various furfuryl or tetrahydrofurfurylamines required for the preparation of such compounds may be prepared in accordance with procedure already known and described in the patent literature. For example, furfurylamine, di-furfurylamine, tetrahydrofurfurylamine and di-tetrahydrofurfurylamine may be prepared as described in U. S. Patents 2,047,926 and 2,045,574. The alkoxy alkylamines may be prepared as described in U. S. Patent 2,285,419.

#### Example 1.—N-furfuryl palmityl amide

Furfurylamine is treated in water with one mole of palmityl chloride and one mole of sodium hydroxide. The product which is the N-furfuryl palmityl amide separates as a light-colored viscous oil which is removed from the reaction mixture, washed with water and dried. The product has the formula



By following the procedure outlined in the preceding paragraph any desired carboxylic amide may be prepared by employing the various furfuryl or tetrahydrofurfurylamines. In some cases, instead of employing the acid chloride, it may be desirable to employ the acid itself or glycerides of such acids as they are found in naturally-occurring oils. If one employs olive oil, or coconut oil, for example, the acids will be present in such oils as a mixture of glycerides and the resulting furfuryl or tetrahydrofurfuryl amides obtained will be a mixture of amides corresponding to the acids

or glycerides thereof which may be present in the oil. Thus there may be prepared a large number of various amide compounds among which may be mentioned the following:

- 5      N-furfuryl stearyl amide  
 N-furfuryl oleyl amide  
 N-furfuryl palmityl amide  
 N-furfuryl naphthenyl amide  
 10     N-furfuryl lauryl amide  
 N-furfuryl decyl amide  
 N-furfuryl ceretyl amide  
 N-furfuryl sebacamide  
 N-difurfuryl stearyl amide  
 15     N-difurfuryl oleyl amide  
 N-difurfuryl palmityl amide  
 N-difurfuryl naphthenyl amide  
 N-difurfuryl lauryl amide  
 N-difurfuryl decyl amide  
 20     N-difurfuryl ceretyl amide  
 N-difurfuryl myristyl amide  
 N-difurfuryl abietyl amide  
 N-difurfuryl benzoyl amide  
 N-ditetrahydrofurfuryl benzoyl amide  
 25     N-ditetrahydrofurfuryl stearyl amide  
 N-ditetrahydrofurfuryl oleyl amide  
 N-ditetrahydrofurfuryl lauryl amide  
 N-ditetrahydrofurfuryl palmityl amide  
 N-ditetrahydrofurfuryl decyl amide  
 30     N-ditetrahydrofurfuryl myristyl amide  
 N-ditetrahydrofurfuryl abietyl amide  
 N-ditetrahydrofurfuryl sebacyl amide  
 N-tetrahydrofurfuryl furfuryl stearyl amide  
 N-tetrahydrofurfuryl furfuryl palmityl amide  
 35     N-tetrahydrofurfuryl furfuryl lauryl amide  
 N-tetrahydrofurfuryl furfuryl oleyl amide  
 N-tetrahydrofurfuryl furfuryl ricinoleyl amide  
 N-tetrahydrofurfuryl furfuryl naphthenyl amide  
 N-tetrahydrofurfuryl furfuryl benzoyl amide  
 40     N-tetrahydrofurfuryl furfuryl abietyl amide  
 N-tetrahydrofurfuryl furfuryl sebacyl amide  
 N-tetrahydrofurfuryl furfuryl ceretyl amide  
 N-tetrahydrofurfuryl methyl palmityl amide  
 N-tetrahydrofurfuryl ethyl lauryl amide  
 45     N-tetrahydrofurfuryl butyl oleyl amide  
 N-tetrahydrofurfuryl cyclohexyl myristyl amide  
 N-tetrahydrofurfuryl amyl naphthenyl amide  
 N-tetrahydrofurfuryl phenyl abietyl amide  
 N-tetrahydrofurfuryl phenyl stearyl amide  
 50     N-tetrahydrofurfuryl phenyl lauryl amide  
 N-tetrahydrofurfuryl lauryl lauryl amide  
 N-tetrahydrofurfuryl beta-hydroxyethyl lauryl amide  
 N-tetrahydrofurfuryl beta-hydroxyethyl stearyl amide  
 55     N-tetrahydrofurfuryl beta-hydroxyethyl palmityl amide  
 N-tetrahydrofurfuryl beta-hydroxyethyl sebacyl amide  
 60     N-tetrahydrofurfuryl beta-hydroxyethyl naphthenyl amide  
 N-tetrahydrofurfuryl beta-hydroxyethyl oleyl amide  
 N-tetrahydrofurfuryl beta-hydroxypropyl oleyl amide  
 65     N-tetrahydrofurfuryl beta-hydroxypropyl palmityl amide  
 N-tetrahydrofurfuryl glyceryl palmityl amide  
 N-furfuryl glyceryl palmityl amide  
 70     N-furfuryl beta-hydroxyethyl palmityl amide  
 N-furfuryl beta-hydroxypropyl palmityl amide  
 N-furfuryl beta-hydroxypropyl oleyl amide  
 N-furfuryl beta-hydroxyethyl lauryl amide  
 N-furfuryl methyl lauryl amide  
 75     N-furfuryl methyl palmityl amide

N-furfuryl ethyloleyl amide  
 N-furfuryl ethyl benzoyl amide  
 N-furfuryl butyl naphthenyl amide  
 N-furfuryl amyl palmityl amide  
 N-furfuryl cyclohexyl stearyl amide  
 N-furfuryl phenyl stearyl amide  
 N-furfuryl phenyl palmityl amide  
 N-furfuryl phenyl ricinoleyl amide  
 N-furfuryl lauryl ricinoleyl amide  
 N-furfuryl lauryl oleyl amide  
 N-furfuryl lauryl palmityl amide  
 N-furfuryl lauryl naphthenyl amide  
 N-furfuryl cetyl naphthenyl amide

*Example 2*

In general, the primary and secondary amines are caused to form amides of ricinoleic acid by heating the acid or its methyl ester with the amine, or by using castor oil, as follows. One mole of difurfurylamine is heated at 100-150° with one mole of methyl ricinoleate. The reaction is preferably carried out in the absence of oxygen or in the presence of an inert gas such as nitrogen. As the reaction proceeds methanol is distilled off and when no more methanol is formed, the reaction is completed. The product, which is a light yellow, heavy viscose oil is washed with water and dried. The product is sufficiently pure for use as an ingredient of a textile yarn treating composition. The product thus prepared is difurfuryl ricinoleyl amide and has the graphic formula



*Example 3*

A mixture of the amides of the various acids present in naturally-occurring oils, such as olive, neat's-foot, teaseed, whale, cotton seed, soyabean, egg, menhaden and other oils, may be prepared in a manner analogous to that described in Examples 1 and 2, that is, by heating the oil, preferably in the absence of oxygen, to a temperature of 100-150° C. For example, one mole of tetrahydrofurfurylamine is mixed with 500 grams of olive oil and heated to a temperature of 150-175° for a period of about two hours. The product which is a heavy, viscous, colorless oil is washed with water and the product which separates at this point is of sufficient purity for use as a yarn conditioning agent. The product is a mixture of amides having the general formula:



wherein R represents a long-chain alkyl group.

*Example 4*

177 grams of difurfurylamine is heated to a temperature of 100-150° C. in a flask fitted with a condenser. 110 grams of acetic anhydride is added slowly and the reaction permitted to proceed for a period of one hour. When the reaction is completed any excess acetic acid is distilled off and the product, which is a heavy, viscous oil is distilled under reduced pressure. The product is N-di-furfurylacetamide having the graphic formula



Following the procedure above described various other furfuryl and difurfuryl amine derivatives may be prepared among which may be mentioned the following.

- 5 N-acetyl furfuryl amine  
 N-propionyl furfuryl amine  
 N-butyryl furfuryl amine  
 N-valeryl furfuryl amine  
 N-beta-methoxyacetyl furfuryl amine  
 10 N-beta-butoxyacetyl furfuryl amine  
 N-acetyl difurfuryl amine  
 N-propionyl difurfuryl amine  
 N-butyryl difurfuryl amine  
 N-valeryl difurfuryl amine  
 15 N-caproyl difurfurylamine  
 N-caproyl ditetrahydrofurfurylamine  
 N-butyryl ditetrahydrofurfurylamine  
 N-propionyl ditetrahydrofurfurylamine  
 20 N-crotonyl ditetrahydrofurfurylamine  
 N-acryl ditetrahydrofurfurylamine  
 N-acetyl ditetrahydrofurfurylamine  
 N-acetyl furfuryltetrahydrofurfurylamine  
 N-lactyl furfuryltetrahydrofurfurylamine  
 25 N-butyryl furfuryltetrahydrofurfurylamine  
 N-butyryl furfuryl ethyl amine  
 N-propionyl furfuryl ethyl amine  
 N-acetyl furfuryl ethyl amine  
 N-acetyl furfuryl butyl amine  
 N-acetyl furfuryl cetyl amine  
 30 N-acetyl furfuryl lauryl amine  
 N-acetyl furfuryl phenyl amine  
 N-acetyl furfuryl-beta-hydroxyethylamine and acetate  
 N-acetyl tetrahydrofurfuryl methylamine  
 35 N-acetyl tetrahydrofurfuryl ethylamine  
 N-acetyl tetrahydrofurfuryl butyrylamine  
 N-acetyl tetrahydrofurfuryl cyclohexylamine  
 N-acetyl tetrahydrofurfuryl naphthenylamine  
 N-acetyl tetrahydrofurfuryl laurylamine  
 40 N-acetyl tetrahydrofurfuryl cetylamine  
 N-lactyl tetrahydrofurfuryl cetylamine  
 N-butyryl tetrahydrofurfuryl laurylamine  
 N-valeryl tetrahydrofurfuryl decylamine  
 45 N-valeryl tetrahydrofurfuryl cyclohexylamine

**YARN LUBRICATING AND ANTI-STATIC TREATMENT**

Our invention will be more readily understood by reference to the following specific examples of typical yarn treating compositions which may be applied to yarns, filaments or fibers to condition them for various textile operations such as knitting, weaving, spinning and the like.

*Example 5*

- 55 N-difurfurylstearyl amide is applied to textile materials (silk, wool, cotton, nylon, viscose, cellulose acetate, Vinyon, etc.) by means of a bath, wick, roller, spray, etc., to facilitate their knitting, weaving, spinning, and the like. If the yarn is intended primarily for knitting the amount of conditioning liquid applied may vary from 2 to 25% by weight of the yarn. If the yarn is intended primarily for weaving the amount of conditioning liquid applied may vary between 1 and 65% of the weight of the yarn.

*Example 6*

- 70 N-difurfuryllauryl amide is applied to textile materials (cellulose acetate, wool, nylon, Vinyon, cotton, viscose, etc.) from a benzene solution as in Example 5. The benzene is then removed by passing the materials through a suitable drying cabinet. As in Example 5, the amount of the composition applied to the textile material will 75 be determined by the use to which the yarn is

to be put or the particular textile operation it is desired to facilitate.

*Example 7*

A conditioning liquid is made up as follows:

|                                   | Parts |
|-----------------------------------|-------|
| Olive oil                         | 99- 1 |
| N-ditetrahydrofurfuryl oleylamide | 1-99  |

This is applied to textile materials such as silk, wool, cellulose acetate and the like as described in Example 5. Cellulose acetate filaments or fibers treated as described above are quite soft and pliable and give improved results in various textile operations such as weaving, knitting and spinning.

Other examples of yarn conditioning compositions which may be applied to various types of yarns, particularly those composed of or containing organic derivatives of cellulose such as cellulose acetate, cellulose propionate, cellulose butyrate, cellulose acetate propionate, cellulose acetate butyrate, cellulose ethers, viscose and other cellulosic materials to lubricate and deelectrify such yarns and render them amenable to a variety of textile operations such as knitting, weaving, spinning and the like are the following.

*Example 8*

|                             | Parts |
|-----------------------------|-------|
| N-furfurylnaphthylamide     | 75-99 |
| Beta-methoxyethyl succinate | 25- 1 |

*Example 9*

|                                    | Parts |
|------------------------------------|-------|
| N-tetrahydrofurfuryl palmitylamide | 75-99 |
| Tetrahydrofurfuryl formal          | 25- 1 |

*Example 10*

|                              | Parts |
|------------------------------|-------|
| N-furfurylcetyl acetyl amide | 1-99  |
| Blown olive oil              | 99- 1 |

*Example 11*

|                                             | Parts |
|---------------------------------------------|-------|
| N-tetrahydrofurfurylcyclohexylstearyl amide | 1-40  |
| Neat's-foot oil                             | 99-60 |

*Example 12*

|                                           | Parts |
|-------------------------------------------|-------|
| N-furfuryltetrahydrofurfurylabietyl amide | 1-50  |
| Blown neat's-foot oil                     | 99-50 |

*Example 13*

|                               | Parts |
|-------------------------------|-------|
| N-ethylfurfuryl ceretyl amide | 1-99  |
| Sperm oil                     | 99- 1 |

*Example 14*

|                           | Parts |
|---------------------------|-------|
| Glycerylacetone acetate   | 10    |
| Butyl stearate            | 20    |
| N-difurfurylbutyryl amide | 10    |
| Blown sperm oil           | 60    |

*Example 15*

|                            | Parts |
|----------------------------|-------|
| N-difurfuryl palmitylamide | 1-30  |
| Mineral oil                | 99-70 |

*Example 16*

|                                             | Parts |
|---------------------------------------------|-------|
| Mineral oil                                 | 30    |
| N-tetrahydrofurfurylphenylsulfoacetyl amide | 30    |
| Blown neat's-foot oil                       | 30    |
| Oleyl alcohol                               | 5     |
| Tetrahydrofurfuryltetrahydrofuroate         | 5     |

*Example 17*

|                             | Parts |
|-----------------------------|-------|
| Mineral oil                 | 70-50 |
| Oleic acid                  | 1-25  |
| 5 N-difurfuryl acetyl amide | 29-25 |

*Example 18*

|                          | Parts |
|--------------------------|-------|
| Mineral oil              | 25    |
| Olive oil (eladized)     | 50    |
| Oleic acid               | 10    |
| Difurfurylamine stearate | 5     |
| Butyl stearate           | 10    |

*Example 19*

|                                               | Parts |
|-----------------------------------------------|-------|
| 15 Blown sperm oil                            | 50    |
| Mineral oil                                   | 30-10 |
| N-difurfuryl ricinoleyl amide                 | 16- 5 |
| 20 Ethyl (mono) phosphate diethanolamine salt | 1-10  |
| Sodium sulfate                                | 2- 0  |
| Oleic acid                                    | 1-25  |

*Example 20*

|                              | Parts |
|------------------------------|-------|
| 25 Beta-methoxyethyl adipate | 20    |
| Blown neat's-foot oil        | 30    |
| Sulfonated olive oil         | 10    |
| Mineral oil                  | 10    |
| Oleic acid                   | 10    |
| 30 Ethanolamine              | 3     |
| Water                        | 7     |
| N-difurfurylstearyl amide    | 10    |

*Example 21*

35 A 20% solution of cellulose acetate in acetone in which is incorporated 1-25% by weight of the cellulose acetate of N-furfurylbutyloleyl amide is extruded through fine orifices into an evaporative atmosphere. The filaments thus produced are wound, or twisted and wound. Yarns produced from filaments thus prepared are pliable and suitable for knitting.

While we have chosen to illustrate our invention by reference to compositions designed primarily for the lubrication, softening, and anti-static conditioning of textile yarns to adapt them for various operations such as knitting, weaving, spinning and the like, the compounds which contribute these valuable properties to yarn treating compositions may also be employed as emulsifying, wetting, and dispersing agents, dye assistants, soaps and for other purposes in which a surface-active agent is required. However, such compounds find their most valuable application in the conditioning of textile yarns, particularly those composed of or containing cellulose organic acid esters such as cellulose acetate, cellulose propionate, cellulose butyrate, cellulose acetate propionate, cellulose acetate butyrate, as well as other cellulosic materials such as viscose, cellulose ethers and the like.

The particular method of application of the yarn treating compositions of our invention to the yarn will depend largely upon the nature of the yarn and the use for which it is intended. In general, the compositions may be applied by any of the standard procedures such as roll, wick, bath, or spray application. If the yarn is in continuous filament form, compositions may be applied just as the yarn emerges from the spinning cabinet, or while passing from package to package. Likewise, the lubricant may be applied during twisting, winding, creping or similar operations. In the case of cut staple fibers, the compositions may be conveniently applied in the form

of an emulsion bath or spray, preferably after any desired special treatment of the yarn such as crimping or the like. In some cases, the lubricating, softening and anti-static agent may be added to the spinning solution from which the yarn is to be spun.

The amount of the compositions applied will, in general, depend upon the purpose for which the yarn is to be used. For example, if the yarn is to be employed for knitting, anywhere from 5-25%, based on the dry weight of the yarn, may be applied. On the other hand, if the yarn is intended for weaving, the amount will generally run from about 1-5%.

In each of the compositions given, the essential lubricating, softening and anti-static component is a compound of the type indicated above. However, as illustrated by the specific examples, such compositions may contain other lubricating, softening, or anti-static agents to augment or supplement the effect of the primary ingredient and thus give the compositions added or improved properties. Likewise, solvents, non-solvents, blending agents, co-solvents, emulsifying agents, dispersing agents and similar ingredients may be added as circumstances may require to adapt the compositions for specific uses. Similarly, various dyes or other coloring matter may be added to the compositions in case it is desired to permanently or fugitively tint the yarn undergoing treatment.

Although in the above examples we have referred to compositions containing specific proportions of the various ingredients, the amounts employed in any given case may vary widely depending upon the particular purpose for which the composition is intended. For example, if it is desired to control the solvent, softening, or other specific action of the conditioning agent per se or of any other ingredient, the amount thereof may be adjusted in accordance with the desired action.

While we have found it convenient to describe our invention with particular reference to the treatment of yarns composed of or containing organic derivatives of cellulose, particularly cellulose acetate, the conditioning agents and compositions described herein are also applicable to the conditioning of many other types of cellulose derivative yarns, such as those composed of or containing cellulose propionate, cellulose butyrate, cellulose acetate propionate, cellulose acetate butyrate, the cellulose ethers such as ethyl, methyl and benzyl celluloses, viscose and couprammonium cellulose, silk, wool, cotton and other natural and artificial materials.

The term "yarn" as used herein and in the claims is to be understood as covering single filaments, a plurality of filaments associated in the form of roving, threads and the like, either of high or low twist, composite threads or yarns composed of a mixture of natural and artificial filaments, composite threads formed by twisting together individual threads or strands of the same or different natural or artificial materials of the same or different deniers, creped or crimped yarns, and crimped or uncrimped cut staple fibers produced from natural or artificial filaments, and spun yarn produced from such staple fibers.

The yarn conditioning methods and compositions of our invention possess many outstanding advantages. The fundamental and distinguishing characteristic of the agents described herein is their ability to lubricate, soften and give val-

able anti-static properties to yarns, particularly those composed of or containing organic derivatives of cellulose such as cellulose acetate, and to render them amenable to various textile operations. These agents are especially valuable in the anti-static treatment of cellulose derivative cut staple fibers.

Among the various yarn treating compositions herein described, we have found that N-furfuryl palmityl amide, difurfuryl ricinoleyl amide and the mixed amides derived from naturally-occurring oils by the procedure outlined in Example 3 are of outstanding value as lubricating and anti-static agents in the conditioning of textile yarns, particularly those composed of or containing cellulose acetate and similar cellulose organic derivatives.

What we claim and desire to secure by Letters Patent of the United States is:

1. The process of conditioning textile yarns comprising an organic derivative of cellulose to render the yarn amenable to textile operations including knitting, weaving, spinning and the like which comprises applying thereto a lubricating and anti-static composition containing as its essential lubricating and anti-static component a carboxylic amide having the formula



wherein Ac is an unsubstituted acyl group, R<sub>1</sub> is a member of the group consisting of furfuryl and tetrahydrofurfuryl groups and R<sub>2</sub> is a member of the group consisting of hydrogen, alkyl, hydroxyalkyl, furfuryl and tetrahydrofurfuryl groups.

2. The process of conditioning textile yarns comprising cellulose acetate to render the yarn amenable to textile operations including knitting, weaving, spinning and the like which comprises applying thereto a lubricating and anti-static composition containing as its essential lubricating and anti-static component a carboxylic amide having the formula



wherein Ac is an unsubstituted acyl group, R<sub>1</sub> is a member of the group consisting of furfuryl and tetrahydrofurfuryl groups and R<sub>2</sub> is a member of the group consisting of hydrogen, alkyl, hydroxyalkyl, furfuryl and tetrahydrofurfuryl groups.

3. Textile yarns comprising organic derivatives of cellulose which are amenable to textile operations including knitting, weaving, spinning and the like, impregnated with a lubricating and anti-static composition containing as its essential lubricating and anti-static component a carboxylic amide having the formula



wherein Ac is an unsubstituted acyl group, R<sub>1</sub> is a member of the group consisting of furfuryl and tetrahydrofurfuryl groups and R<sub>2</sub> is a member of the group consisting of hydrogen, alkyl, hydroxyalkyl, furfuryl and tetrahydrofurfuryl groups.

4. Textile yarns comprising cellulose acetate which are amenable to textile operations including knitting, weaving, spinning and the like, impregnated with a lubricating and anti-static composition containing as its essential lubricating and

anti-static component a carboxylic amide having the formula



wherein Ac is an unsubstituted acyl group, R<sub>1</sub> is a member of the group consisting of furfuryl and tetrahydrofurfuryl groups and R<sub>2</sub> is a member of the group consisting of hydrogen, alkyl, hydroxyalkyl, furfuryl and tetrahydrofurfuryl groups.

5. The process of conditioning textile yarns comprising an organic derivative of cellulose to render the yarn amenable to textile operations 15

including knitting, weaving, spinning and the like which comprises applying thereto a lubricating and anti-static composition containing as its essential lubricating and anti-static component N-furfuryl palmityl amide.

6. Textile yarns comprising cellulose acetate which are amenable to textile operations including knitting, weaving, spinning and the like, impregnated with a lubricating and anti-static composition containing as its essential lubricating and anti-static component N-furfuryl palmityl amide.

JOSEPH B. DICKEY.  
JAMES G. McNALLY.